

## UNITED STATES PATENT OFFICE

ERICH RICHTER, OF WOLFEN, GERMANY, ASSIGNOR TO I. G. FARBENINDUSTRIE AKTIENGESELLSCHAFT, OF FRANKFORT-ON-THE-MAIN, GERMANY

## CIGARETTE TIP COIL

No Drawing. Application filed June 18, 1926, Serial No. 116,984, and in Germany March 18, 1925.

This invention relates to material for use as cigarette tips and particularly to material, or rolls thereof, which may be used in cigarette-making machines.

5 In the cigarette industry extremely thin films consisting of metal powder and cellulose derivatives are widely used as substitutes for metal foil as coverings for the tips of cigarettes. The metal-containing films, 10 after production in wide strips, are cut into narrow strips and rolled together with paper strips of the same width into so-called coils or rolls.

During the manufacture in the cigarette 15 machine these rolls have been proven defective by reason of the fact that they are easily electrified. This arises chiefly from the thin film, partly also from the paper which serves as a base for the latter. As the process of 20 manufacture is carried out in a relatively dry atmosphere the foil and paper take up a charge of static electricity as they are unwound from the coil, which electrical charge exerts an injurious influence on the subsequent steps of production.

An object of the present invention is to provide a tipping coil free from the defects noted above and which will run smoothly through and may be accurately and positively guided in the cigarette tipping machine. More specifically, an object is to provide a coil in which the metal-containing film and/or the paper have such properties that injurious charges of static electricity cannot 35 be established.

With the foil or film this is accomplished by using therefor a cellulose derivative which per se is non-static, i. e. is not electrifiable, or admixtures of cellulose derivatives 40 which, individually electrifiable, are non-static in admixture. Another possibility consists in giving an electrically excitable foil a well conducting addition, for example, hygroscopic substances, such as glycerine, certain salts and the like, so that the film or foil becomes a good conductor. A particularly advantageous manner of securing the conductivity is to employ the metal powder in such high proportion as to give the composite 45 film the desired degree of conductivity. The

desired property is imparted to the paper in a most simple manner by saturating with hygroscopic substances, although other means may be used for preventing the paper from taking on an electrical charge. 55

The following examples indicate typical methods of preparing coils in accordance with the invention:

(1) Add while well stirring 3 to 4 parts of bronze to 7 parts of a 20 percent solution 60 of cellulose acetonitrile, containing from 2 to 3 percent of nitrogen, in the usual solvents with an addition of one or more of the well known plasticizers in the amount of 5 percent. After filtration the solution is spread in the 65 usual way on a flowing apparatus familiar to those skilled in the art. The film thus produced is wound to cigarette tip coils which when being worked in cigarette machines do not take up any electrostatic charge. 70

(2) Add 3 to 4 parts of bronze to 7 parts of a 20 percent solution of a mixture of two parts of ethyl cellulose and 1 part of nitrocellulose in the usual solvents and with an addition of one or more of the usual plasticizers 75 in the amount of 5 percent. This solution is worked in the way described above. The cigarette-tip coil produced does not take up electrostatic charges.

(3) On taking off the film from the flowing 80 apparatus paper is wound into its windings. The paper used for this purpose is previously soaked in a 0.5 percent solution of ammonium chloride, passed through a drying channel and rewound. Cigarette-tip coils manufactured with this paper do not collect electrostatic charges even when the film itself is not made antistatic. 85

Coils or rolls embodying the invention may be employed in the manufacture of cigarettes 90 by machinery with complete freedom from the difficulties which have been experienced with coils which were electrifiable.

## Claims:

1. A cigarette tip coil of the type comprising 95 a strip film of cellulosic material and metal powder, and a paper strip, characterized by the fact that both the film and the strip are formed of materials which do not retain electric charges.

2. A cigarette coil as defined in claim 1, wherein one of said strips includes hygroscopic material in quantity sufficient to render the strip conductive.
5. The invention as claimed in claim 1, wherein said cellulosic material comprises a plurality of cellulosic derivatives, which are individually electrifiable.

In testimony whereof, I affix my signature.  
10 **ERICH RICHTER.**

**15****20****25****30****35****40****45**